

# United States Patent Office

3,111,434

Patented Nov. 19, 1963

1

3,111,434

## SURFACE HARDENING OF METAL BODY CONSISTING OF OR CONTAINING TITANIUM OR ZIRCONIUM

Zenichiro Takao, Nishinomiya, and Shigeo Inomata and Koichi Nakano, Higashinada-ku, Kobe, Japan, assignors to Kobe Steel Works, Ltd., Kobe, Japan  
No Drawing. Filed Aug. 1, 1960, Ser. No. 46,351  
4 Claims. (Cl. 148—13.1)

The present invention relates to surface hardened metal bodies or articles consisting of or containing titanium or zirconium, and also to a process for surface hardening metal bodies or articles consisting of or containing titanium or zirconium.

The metals belonging to the titanium group of the periodic system, particularly titanium, zirconium and alloys containing the same have relatively low specific gravities and are excellent in tensile strength and anti-corrosive properties, and therefore have extensively been used as materials for various articles, structures, apparatus, etc. including chemical apparatus and appliances. However, titanium and zirconium are low in hardness and are poor in wear resistance and furthermore have drawbacks that they are damaged particularly when applied to those which are subjected to friction. For these reasons, these materials are not fully satisfactory in spite of their various excellent properties.

It is an object of the present invention to provide surface hardened metal bodies or articles consisting of or containing titanium or zirconium which show excellent wear resistance and antifriction due to the hardened surface layer.

It is another object of the present invention to provide a process for surface hardening metal bodies or articles consisting of or containing titanium or zirconium to render them wear resistant and antifriction to make them more useful.

In accordance with the invention, an improved metal body or article consists of a base metal consisting of or containing titanium or zirconium and a surface hardened coating or layer which consists of the nitride and/or oxide of the metal or alloy of the said base, or consists of a dispersed layer of the nitride and/or oxide.

The hardened surface coating or layer is formed by reacting the surface layer of the base metal or alloy with oxygen and/or nitrogen. It is preferable to use gaseous oxygen and gaseous nitrogen as oxidizing and nitridation agents respectively. More particularly, according to the present invention, the nitride and/or oxide are formed by utilizing the so-called inert gas shielded arc welding arrangement with or without a filler metal rod consisting of the same material as the base metal or alloy. Oxygen and/or nitrogen gas are mixed with the inert gas so that the nitridation and/or oxidation occur while the surface is being covered by the inert gas. When the filler metal is not used the surface of the base is reacted with oxygen and/or nitrogen to integrally form the oxide and/or nitride thereon, while when the filler metal is used the molten filler metal itself forms the oxide and/or nitride layer or coating on the base.

Titanium is chemically stable below 500° C. but becomes very active at higher temperatures and reacts with oxygen at temperatures higher than the red heat (500° C.) to form titanium oxide as a solid solution or dispersion layer consisting mainly of titanium dioxide, and reacts with nitrogen at temperatures higher than 860° C. to form a solid solution or dispersion layer of titanium nitride. In this connection it should be noted that solubility of oxygen and nitrogen in titanium is appreciably higher than in other practical metals. Similarly, zirconium reacts with oxygen and nitrogen at elevated tempera-

2

tures (500° C.). The same is true in respect to titanium or zirconium base alloys. In any case, the oxide and/or nitride forms very hard surface layer or coating on the base metal or alloy.

According to the present invention, the formation of the desired oxide and/or nitride is effected by shielding the surface of the base metal body or article with an inert gas such as argon or helium and the surface is arc molten or coated with additional molten metal (by using a filler metal rod) while introducing a predetermined amount of oxygen and/or nitrogen in the inert gas.

As is known, atmospheric air is abundant with oxygen and nitrogen and it is apparent that when air is employed oxygen and nitrogen as contained therein serve as reactive gas to form the oxide and nitride. Simply considered, the use of atmospheric air may be convenient and economical. However, it has been found that the same is not true from the practical point of view. That is, the flow of air into the reaction zone is very unstable and nonuniform and in addition thereto arc producing condition such as electric current is not constant at all times and usually varies from instant to instant, so that the formed oxide and nitride are nonuniform in the extent and structure.

Therefore, according to the invention it is preferable not to use atmospheric air but to introduce into the inert gas separately prepared oxygen and/or nitrogen. Thus, the amount and proportions of oxygen and/or nitrogen can be controlled quite easily as desired to stabilize the oxidation and/or nitridation reaction and form the desired and uniform hardened surface.

As mentioned hereinbefore, it is preferable to employ an inert gas shielded arc welding arrangement which, so well known to those skilled in the art as requiring no detailed explanation, is a shield arc welding carried out in an inert gaseous atmosphere. As is conventional, an electrode of material having a high melting point such as tungsten is employed. When the hardened layer to be formed is relatively thin ( $\frac{1}{100}$ — $\frac{1}{100}$  mm. or less), no filler metal rod is used and the surface to be hardened is arc molten and reacted with oxygen and/or nitrogen while shielded with the inert gas to form the hard oxide and/or nitride. If the hardened layer to be formed is relatively thick (up to 5 mm. or thicker), it is preferable to use a filler metal in the usual manner. The filler metal which is the same material as the base metal to be coated is similarly arc molten and reacted with oxygen and/or nitrogen while shielded with the inert gas to form the hard oxide and/or nitride which are deposited on the said surface.

It is apparent that the amount of oxygen and/or nitrogen to be supplied in the inert gas will largely control the hardness of the formed layer or coating. Thus, when the amount of the reactive gas is less than that required no sufficient hardness would be obtained, while if the amount of the reactive gas is excessive fragility of the oxide and/or nitride is unduly increased so that the surface would become brittle.

The amount of the reactive gas is selected depending upon the desired hardness to be accomplished, the particular metal or alloy from which the body or article is formed, and the thickness of the hardened layer or coating. This amount can be selected easily by those skilled in the art by means of a small scale pretesting. The amount of the reactive gas (oxygen and/or nitrogen) is determined by the proportion occupying in the inert gas. Generally, when the metal surface itself is molten and hardened without using a metal deposition from the filler metal rod it has been found that the amount of the reactive gas is preferable to be selected less than 15% by volume of the inert gas, while when the metal deposition is used the amount of the reactive gas is preferable to

be less than 10% by volume of the inert gas. In the latter case the said less amount is caused by the use of the filler metal rod for the deposition coating. That is, when such filler metal rod is employed atmospheric air comes to get mixed in even if the inert gas shield is established, and oxygen and nitrogen contained in this air would take part in the reaction so that this must be taken into consideration beforehand.

Generally, the weld or arc current is preferable to be controlled within the range from 60 to 130 amp., although not absolutely necessary to be limited to this particular range. The arc length usually is about 2-10 mm. The flow of the inert gas such as argon or helium to establish the inert gas atmosphere or shield around the portion to be welded or molten may, in most cases, be about 10-30 ft.<sup>3</sup>/hr.

The oxide and/or nitride solid solution layer or dispersion layer or deposition coating thus formed on the base metal body or article is very uniform and generally has hardness of from 250 to 550 as measured by Vickers hardness meter (load 30 kgs.).

According to this invention, since the reactive gas (oxygen and/or nitrogen) is introduced in the inert gas which creates an inert gas shield the stability and uniformity of the reaction are assured, the control of the reaction is easy so that there is obtained a uniform hard layer or coating. By using the filler metal rod for deposition a thick coating, if desired, can be obtained. In this case, by controlling the amount of the deposition, the thickness of the hard coating may be varied as desired. Furthermore, since the definite or calculated amount of oxygen and/or nitrogen can be introduced, and undesired intrusion of atmospheric air (which would cause nonuniformity of the formed layer or coating) is prevented by the inert gas shield, the layer or coating formed is substantially uniform in hardness and structure or composition.

The invention will be further described with reference to the following examples. However, it should be understood that these examples are for illustration only and not for limiting the invention in any way.

#### Example 1

A titanium rod circular in cross section and 17 mm. in diameter was surface hardened by depositing a titanium oxide layer thereon. A usual inert gas shielded arc welding apparatus with tungsten electrode was employed together with a filler titanium rod for the deposition. In the first the weld deposition was carried out by using usual or common argon gas (oxygen content 0%). Next, the same procedure was repeated with the use of sigma grade argon gas (oxygen content 5%), and finally with a mixture of equal amount of argon gas and sigma grade gas, the oxygen content in said mixture being 3.4% ac-

cording to gas analysis. In any case, the welding conditions were equally as follows:

|                 |                          |
|-----------------|--------------------------|
| Welding current | 75-95 amp.               |
| Arc voltage     | 8-9 v.                   |
| Arc length      | 3-4 mm.                  |
| Gas flow        | 15 ft. <sup>3</sup> /hr. |
| Welding speed   | 100-130 mm./min.         |

In each case the deposition coating or layer was formed in thickness of 5 mm. and its hardness was remarkably higher than that of the base metal or titanium.

#### Example 2

In this example, bodies of titanium, titanium base alloys, zirconium, and zirconium base alloys were surface hardened by employing an oxygen and/or nitrogen gas mixed inert gas shielded arc welding arrangement without using a filler metal, under various conditions. The results were as indicated in the following table. In any case, the surface hardness was measured by Vickers hardness meter (load 30 kgs.).

| Body     | Weld current (amp.) | Arc length (mm.) | Argon gas (ft. <sup>3</sup> /hr.) | Reactive gas, percent | Weld speed (mm./min.) | Surface hardness |
|----------|---------------------|------------------|-----------------------------------|-----------------------|-----------------------|------------------|
| Ti       | 60-150              | 2-10             | 10-30                             | 30 (O <sub>2</sub> )  | 100-150               | 250-600          |
| Ti alloy | 60-150              | 2-10             | 10-30                             | 30 (O <sub>2</sub> )  | 100-150               | 250-600          |
| Zr       | 60-180              | 2-10             | 10-30                             | 30 (O <sub>2</sub> )  | 100-150               | 250-600          |
| Zr alloy | 60-180              | 2-10             | 10-30                             | 30 (O <sub>2</sub> )  | 100-150               | 250-600          |

#### Example 3

In this example, titanium and titanium alloy base bodies were surface hardened by depositing a titanium oxide and nitride layer thereon. A usual inert gas shielded arc welding apparatus with tungsten electrode was employed together with a filler metal rod as indicated for the deposition. The result was as follows:

| Body     | Weld current (amp.) | Arc length (mm.) | Argon gas (ft. <sup>3</sup> /hr.) | Reactive gas, percent | Filler metal | Surface hardness |
|----------|---------------------|------------------|-----------------------------------|-----------------------|--------------|------------------|
| Ti       | 60-150              | 2-10             | 10-30                             | 20 (O <sub>2</sub> )  | Ti           | 300-500          |
| Ti       | 60-150              | 2-10             | 10-30                             | 20 (O <sub>2</sub> )  | Ti alloy     | 350-500          |
| Ti alloy | 60-150              | 2-10             | 10-30                             | 20 (O <sub>2</sub> )  | Ti alloy     | 350-500          |
| Ti alloy | 60-150              | 2-10             | 10-30                             | 20 (O <sub>2</sub> )  | Ti alloy     | 300-500          |

In any case, the welding speed was 100-150 mm./min.

#### Example 4

In this example, various titanium, zirconium and their base alloy bodies listed below were surface hardened by employing an oxygen and/or nitrogen gas mixed inert gas shielded arc welding with or without using a filler metal, under various conditions indicated. The various conditions and results are given below.

| Exp. | Body     | Filler Rod | Shield gas | Reactive Gas, Percent |    | Current (amp.) | Gas flow (l./min.) | Weld Speed (mm./min.) | Length of arc (mm.) |
|------|----------|------------|------------|-----------------------|----|----------------|--------------------|-----------------------|---------------------|
|      |          |            |            | O <sub>2</sub>        | N  |                |                    |                       |                     |
| 1    | Ti       | Ti         | Ar         | 1                     | 0  | 100-130        | 5-10               | 100-130               | 3-4                 |
| 2    | Ti       | Ti         | Ar         | 3                     | 0  | 100-130        | 5-10               | 100-130               | 3-4                 |
| 3    | Ti       | Ti         | Ar         | 6                     | 0  | 100-130        | 5-10               | 100-130               | 3-4                 |
| 4    | Ti       | Ti         | Ar         | 0                     | 1  | 100-130        | 5-10               | 100-130               | 3-4                 |
| 5    | Ti       | Ti         | Ar         | 0                     | 3  | 100-130        | 5-10               | 100-130               | 3-4                 |
| 6    | Ti       | Ti         | Ar         | 0                     | 6  | 100-130        | 5-10               | 100-130               | 3-4                 |
| 7    | Ti       | Ti         | Ar         | 0                     | 10 | 100-130        | 5-10               | 100-130               | 3-4                 |
| 8    | Ti alloy | Ti alloy   | Ar         | 2                     | 0  | 100-130        | 5-10               | 80-120                | 5-8                 |
| 9    | Ti alloy | Ti alloy   | Ar         | 2                     | 0  | 100-130        | 5-10               | 80-120                | 5-8                 |
| 10   | Zr       | Zr         | Ar         | 5                     | 0  | 100-120        | 5-10               | 100-130               | 3-4                 |
| 11   | Zr       | Zr         | Ar         | 0                     | 5  | 100-120        | 5-10               | 100-130               | 3-4                 |
| 12   | Ti       | Ti         | He         | 5                     | 0  | 100-120        | 7                  | 100-130               | 3-4                 |
| 13   | Ti       | -----      | Ar         | 3                     | 0  | 90-130         | 7                  | 100-120               | 3-4                 |
| 14   | Ti       | -----      | Ar         | 6                     | 0  | 90-130         | 7                  | 100-120               | 3-4                 |
| 15   | Ti       | -----      | Ar         | 0                     | 1  | 90-130         | 7                  | 100-120               | 3-4                 |
| 16   | Ti       | -----      | Ar         | 0                     | 6  | 90-130         | 7                  | 100-120               | 3-4                 |
| 17   | Ti       | -----      | Ar         | 0                     | 10 | 90-130         | 7                  | 100-120               | 3-4                 |
| 18   | Zr       | -----      | Ar         | 5                     | 0  | 90-120         | 7                  | 100-120               | 3-4                 |
| 19   | Ti       | Ti         | Ar         | 0                     | 0  | 80-120         | 7                  | 100-120               | 3-5                 |

In the above table, the alloy of Exp. 8 consisted of 0.025% C, 0.065% Fe, 0.05% Si, 1.06% Mo, 4.53% Al, 2% Cr and rest Ti, while the alloy of Exp. 9 consisted of 0.2% C, 0.075% Fe, 0.015% Si, 4.36% Al, 4.54% Mn and rest Ti.

After the welding operation, hardness of these metal bodies was as indicated below, when measured by Vickers hardness meter (load 30 kgs.).

| Exp. No.: | Hardness |
|-----------|----------|
| 1         | 300-350  |
| 2         | 350-460  |
| 3         | 400-550  |
| 4         | 320-350  |
| 5         | 300-400  |
| 6         | 350-480  |
| 7         | 470-550  |
| 8         | 370-450  |
| 9         | 390-510  |
| 10        | 400-550  |
| 11        | 450-550  |
| 12        | 400-550  |
| 13        | 350-400  |
| 14        | 350-450  |
| 15        | 250-300  |
| 16        | 300-420  |
| 17        | 350-500  |
| 18        | 350-400  |
| 19        | 200-250  |

What we claim is:

1. A method of surface-hardening a metal body selected from the group consisting of titanium and zirconium, which comprises the steps of: forming a layer on the surface of the body by reacting said body with a reactive gaseous element in an inert gas-shielded arc welding arrangement by heating the body surface to a temperate at which it is molten, and introducing in the inert gas the reactive gaseous element so that said surface of the body while being arc-welded and shielded by the inert gas, is reacted with said reactive gaseous element to form the layer.

2. A method of surface hardening a metal body selected from the group consisting of titanium, zirconium, and ti-

tanium base alloys, said method comprising the steps of: shielding the body with an inert gas having mixed therewith a measured amount of reactive gas for reacting with the body and simultaneously arc welding the body in the gas shield at a temperature which provides a molten surface on said body so that the molten portion of the body reacts with the reactive gas to form a hard layer on the surface of said body.

3. A method of surface hardening a metal body selected from the group consisting of titanium, zirconium, an alloy of 0.025% C, 0.065% Fe, 0.05% Si, 1.06% Mo, 4.53% Al, 2% Cr and the remainder titanium, and an alloy of 0.2% C, 0.075% Fe, 0.015% Si, 4.36% Al, 4.5% Mn and the remainder titanium, said method comprising the steps of: shielding the body with an inert gas selected from the group consisting of argon and helium, and having mixed therewith a measured amount of reactive gas selected from the group consisting of oxygen and nitrogen for reacting with the body to thereby form a hard oxide and/or nitride layer, said inert gas being supplied at a rate of 10-30 ft.<sup>3</sup> per hour and simultaneously arc welding the body in the gas shield at a temperature which provides a molten surface on said body so that the molten portion of the body reacts with the reactive gas to form a hard layer on the surface of said body.

4. A method as defined in claim 3 comprising depositing metal from a filler metal rod onto the body during arc welding.

30

References Cited in the file of this patent

UNITED STATES PATENTS

1,748,378 Armstrong Feb. 25, 1930  
2,523,883 Strauchen et al. Sept. 26, 1950  
35 2,892,743 Griest et al. June 30, 1959

FOREIGN PATENTS

555,952 Canada Apr. 15, 1958

OTHER REFERENCES

40 Titanium, McQuillan & McQuillan, pages 398-400, Butterworth, Scientific Publications, 1956.  
Morris: Welding Principles for Engineers, page 53.